

Patented Jan. 25, 1927.

## UNITED STATES PATENT OFFICE.

WALTHER EHLERS, OF BERLIN-GRUNAU, GERMANY, ASSIGNOR TO GENERAL ELECTRIC COMPANY, A CORPORATION OF NEW YORK.

## MAGNETIC CORE.

No Drawing. Application filed March 14, 1925, Serial No. 15,697, and in Germany April 10, 1924.

My present invention relates to the construction of magnetic cores such, for example, as those adapted for use in connection with telephone circuits.

5 Magnetic cores formed of compressed mixtures of insulating material and magnetic material have been used to a considerable extent in telephone practice. In the construction of such cores, however, it is practically impossible to produce a uniform compression throughout the entire mass. In practice the edges or outer portions become more compressed than the interior portions and as a result the insulation between the 10 magnetic particles at the outer portions is considerably less than the insulation between the magnetic particles in the interior portions, and the edges or outer portions furnish an unproportionally large percentage of the 15 energy losses because of eddy currents between individual particles.

To overcome this difficulty it has been proposed to form a core by assembling a sufficient number of flat pressed pieces to form 20 the desired body. Such construction, however, greatly increases the cost of manufacture.

The object of my invention is to provide 25 a form of magnetic core in which the disadvantages pointed out may be overcome, and in which the insulation between the magnetic particles at the points subjected to the greatest pressure will be as great as at other 30 points in the core.

35 The object of my invention may be attained in various ways. One way of accomplishing the desired result is to fill different parts of the press form with different mixtures, that is, the mixture in the outer or 40 edge portion of the form may have a greater proportion of insulating material than the mixture in the central, or inner, portion.

On the other hand, different insulating materials may be used for the different mixtures, the mixture used for the outer por-

tions having an insulating material of superior insulating properties to that used in the central portions.

In carrying my invention into effect a wide variety of finely divided insulating materials may be employed, such, for example, as resinous material, glass or various ceramic materials.

Similar results may be obtained by impregnating the pressed body from the outside. By this means the insulation of the outer more highly compressed portions of the core may be increased so as to be substantially as strong as that of the inner portions. The proportion of insulating material present in the outer portion of the core may by this method be increased above that present in the inner portion.

What I claim as new and desire to secure by Letters Patent of the United States, is:—

1. A magnetic core formed of a compressed mixture of magnetic material and insulating material, and having in the densest portions thereof a relatively greater proportion of insulating material than the proportions which are less dense.

2. A magnetic core comprising a compressed mixture of magnetic material and insulating material and having in its outer portions a relatively greater proportion of insulating material than in its inner portion.

3. In the construction of a magnetic core of pressed magnetic material and insulating material the method of compensating for differences in insulation strength due to differences in pressure which consists in providing in the parts subjected to the greatest pressure a relatively greater proportion of insulating material than in the parts subjected to lower pressures.

In witness whereof, I have hereunto set my hand this 17th day of February, 1925.

WALTHER EHLERS.